

## UNITED STATES PATENT OFFICE

2,669,513

TITANIUM BASE ALLOYS CONTAINING  
ALUMINUM AND TIN

Robert I. Jaffee, Worthington, and Horace R. Ogden and Daniel J. Maykuth, Columbus, Ohio, assignors, by mesne assignments, to Rem-Cru Titanium, Inc., Midland, Pa., a corporation of Pennsylvania

No Drawing. Application April 29, 1952,  
Serial No. 285,076

4 Claims. (Cl. 75—177)

1

This invention relates to titanium base alloys and particularly to alloys of titanium with aluminum and tin. The invention further contemplates the addition to a titanium-aluminum-tin base of one or more of numerous substitutional ingredients, among which are antimony, beryllium, bismuth, copper, manganese, silver and zirconium.

The use of titanium as a structural material is limited by its relatively low strength and high cost, and it becomes desirable to alloy titanium with such other metals as will increase the strength to acceptable levels and preferably at the same time effect some reduction in the total material cost. Aluminum is a metal well suited to the attainment of these objectives. It is quite plentiful, has a low density, and has a material strengthening effect on titanium. However, the amount of aluminum alone that can be added to titanium is limited by its adverse effect on ductility. Binary alloys of titanium with more than about 5% of aluminum are too brittle for most structural uses; and such binary alloys containing less than about 5% of aluminum do not possess sufficient strength to be of general utility. A further strengthening, as well as an increase in the amount of relatively inexpensive aluminum, is highly desirable.

The present invention, in one of its aspects, comprises the discovery that the addition to titanium-aluminum alloys of a few percent of tin, effects a marked improvement in the properties of titanium-aluminum alloys of a given aluminum content, say 3.5% to 5%, and likewise enables an increase of the aluminum content up to about 7.5% with a material increase in strength, while maintaining adequate ductility.

The invention further contemplates, in its broader aspect, a series of alloys which may be

2

regarded as additions of aluminum, with or without other ingredients, to a titanium-tin base. The tin content of such alloys may range from about 1% to 23%, with the aluminum ranging from about 0.25 to 7.5% depending on the tin content, the aluminum being preferably on the low side when the tin is on the high side and vice versa. It has been found that these alloys, particularly those of relatively high tin content, not only have excellent properties when made from substantially pure titanium, but are characterized by a most unusual tolerance for the interstitial ingredients, carbon, oxygen and nitrogen. For example, an alloy of 10% tin, 2% aluminum, 0.2% nitrogen, balance titanium, possesses a rare combination of high strength and good ductility.

For producing ductile titanium-tin-aluminum alloys in accordance with the invention, having good forging and rolling properties, the aluminum content is preferably related to the tin content substantially in accordance with the following proportions:

Table I

|           | Tin Content, Percent | Aluminum Content, Percent |
|-----------|----------------------|---------------------------|
| 30 1..... |                      | 0.5-6                     |
| 5.....    |                      | 0.5-5                     |
| 10.....   |                      | 0.5-4.5                   |
| 15.....   |                      | 0.25-4                    |
| 20.....   |                      | 0.25-3                    |
| 23.....   |                      | 0.25-1                    |

The metal used as a base for any of the alloys of the present invention may contain the interstitial contaminants, carbon, oxygen and/or nitrogen, in amounts ranging from 0.02% up to 40 at least the total quantity to be found in good

commercial titanium. Further controlled additions of the interstitials show some distinctive

annealed for 3½ hours at 850° C., unless otherwise noted, are as follows:

Table II

[Iodide titanium-base alloys]

| Composition,<br>Percent (Balance<br>Titanium) |     |     | Tensile Properties: p. s. i. $\times 1,000$ |                         |                      |                           |        |
|-----------------------------------------------|-----|-----|---------------------------------------------|-------------------------|----------------------|---------------------------|--------|
| Al                                            | Sn  | C   | Annealed<br>V. H. N.<br>Surface             | 0.2%<br>Offset<br>Yield | Ultimate<br>Strength | Elongation<br>1", Percent | Bend T |
| 0                                             | 0   |     | 88                                          | 22                      | 37                   | 61 <sup>1</sup>           | 0      |
| 5                                             | 1   |     | 278                                         | 67                      | 78                   | 15                        | 7      |
| 5                                             | 2.5 |     | 312                                         | 81                      | 88                   | 14                        | 1.6    |
| 5                                             | 5   |     | 312                                         | 90                      | 94                   | 12                        | 1.1    |
| 5                                             | 2.5 | .1  | 385                                         | 129                     | 144                  | 12                        | 1.4    |
| 5                                             | 2.5 | .2  | 404                                         | 130                     | 145                  | 12                        | 1.6    |
| 5                                             | 2.5 | .3  | 426                                         | 149                     | 152                  | 3                         | (3)    |
| 5                                             | 2.5 | .35 | 427                                         | 140                     | 144                  | 4                         | (3)    |
| 5                                             | 1.5 | .25 | 394                                         | 140                     | 149                  | 9                         | 4.4    |
| 5                                             | 2   | .25 | 389                                         | 140                     | 161                  | 13                        | 4.2    |
| 5                                             | 3   | .25 | 390                                         | 139                     | 149                  | 13                        | 4.2    |
| 5                                             | 3.5 | .25 | 399                                         | 144                     | 161                  | 11                        | 4.2    |
| 5                                             | 5   | .25 | 391                                         | 144                     | 147                  | 17                        | 2.3    |
| 5                                             | 7.5 | .25 | 398                                         | (3)                     | 110                  | 0                         | 6.2    |
| 17.5                                          | 1   |     | 357                                         | 103                     | 106                  | 20                        | 2.8    |
| 7.5                                           | 2.5 |     | 324                                         | 94                      | 101                  | 16                        | 1.8    |
| 7.5                                           | 5   |     | 357                                         | 109                     | 118                  | 14                        | 7      |
| 7.5                                           | 7.5 |     | 398                                         | 116                     | 116                  | (3)                       | (3)    |
| 27.5                                          | 2.5 | .25 | 392                                         | 136                     | 138                  | 10                        | 2.3    |
| 27.5                                          | 2.5 | .25 | 393                                         | 132                     | 132                  | 9                         | 6      |

<sup>1</sup> Annealed 4 hours at 925° C.<sup>2</sup> Annealed 3½ hours at 850° C. plus 1 hour at 925° C.<sup>3</sup> Brittle.

effects. In general, the tolerance for the interstitials, as determined by a ductility requisite to broad and varied utility, is greater than that of most titanium alloys, and this is particularly true of those alloys which contain a relatively small amount of aluminum. For example, in alloys containing not over 5% tin and not over about 2% aluminum, carbon may be added up to about 1% without excessive embrittlement.

However, increasing the metallic alloy constituents diminishes the carbon tolerance. For example, in an alloy containing say 13% tin and 3% aluminum, balance titanium, the bend ductility deteriorates rapidly if the carbon content is increased above about 0.2%. As distinguished from carbon, the tolerance for nitrogen diminishes more slowly from a maximum of about 0.3% for a very low content of aluminum and tin to a value between 0.15% and 0.19% which remains almost constant for a wide range of compositions. Oxygen occupies an intermediate position, the tolerance therefor decreasing at a more constant rate from a maximum of about 0.5%. The permissible oxygen content of an alloy containing 13% tin, 3% aluminum is about 0.2%.

The alloys of this invention may be prepared by melt-casting in an atmosphere of argon, rolling at a suitable temperature, say 850° C. to 980° C., and annealing under conditions which will effect recrystallization but not substantial grain growth or re-solution of carbides. A typical but by no means universal annealing treatment comprises soaking at a temperature of about 850° C. for from 2 to 3½ hours. The rate of cooling after annealing is not material, since in these alloys the titanium, with the exceptions noted later, is all in the alpha phase except for minor amounts which may be combined as titanium-carbide.

The properties of selected alloys of titanium of requisite purity with aluminum and tin, as

35 In the foregoing table, and those which follow, "bend ductility" is measured as the radius upon which the alloy can be bent without fracture to an angle of 75°, the radius being stated as a multiple of the specimen thickness.

40 Microscopic examination shows most of these alloys to be of small grain size, probably due to a fine distribution of carbides. Carbon is less soluble in beta titanium than in alpha titanium, hence in a melt containing, say 0.2 carbon, a substantial proportion of the carbon will be present as carbides, which as the melt congeals are frozen in a matrix of beta titanium in a fine dispersion. As recrystallization proceeds without substantial solution of carbides, the numerous carbide particles form nucleation sites for the growth of relatively small alpha grains, and inhibit the growth of large grains. Grain sizes as small as 0.012 mm. and 0.015 mm. have been observed repeatedly, and the average grain size is from about 0.020 mm. to 0.030 mm. Fine grain size and the presence of visible carbide particle stringers are associated with the substantial differences between yield strength and ultimate strength appearing in the above table. This characteristic renders the alloys universally useful, being particularly advantageous for sheet and other forms which are stretched in fabrication.

45 All of the alloys whose properties are tabulated in Table II above contain a minimum of 5% of aluminum and show embrittlement by a tin content of about 7.5%. A reduction of the aluminum content, say to 2%, greatly increases the tolerance for tin as well as for the interstitials, enabling the use of as much as 23% tin. For example, an alloy containing 10% tin, 2% aluminum, and 0.2% nitrogen, has a 0.2% offset yield strength of 135,000, an ultimate strength of 142,000, with an elongation of 16% and a bend ductility of 2.1 T.

50 Other alloys containing varying amounts of

55 60 65 70 75 80 85 90 95 100

aluminum, tin and the interstitials, and their properties as rapidly cooled after annealing in

argon for 2 hours at 850° C., are given in Tables III, IV-A and IV-B below:

Table III

[Iodide-titanium-base alloys]

| Composition, Percent<br>(Balance Titanium) |     |      |      | Tensile Properties: p. s. i. × 1,000 |                      |                     |                                 |                                  |                   |
|--------------------------------------------|-----|------|------|--------------------------------------|----------------------|---------------------|---------------------------------|----------------------------------|-------------------|
| Sn                                         | Al  | C    | N    | 0.2%<br>Offset<br>Yield              | Ultimate<br>Strength | Elongation<br>to 1" | Percent<br>Reduction<br>in Area | Annealed<br>Hardness,<br>Vickers | Min.<br>Bend<br>T |
| 1                                          | 1   | --   | --   | 22                                   | 37                   | 61                  | 58                              | 88                               | 0                 |
| 1                                          | 1   | 0.25 | --   | 30                                   | 50                   | 28                  | 55                              | 156                              | 0                 |
| 1                                          | 2   | --   | --   | 34                                   | 53                   | 25                  | 56                              | 251                              | 0.6               |
| 1                                          | 2   | 0.25 | --   | 36                                   | 86                   | 29                  | 46                              | 179                              | 1.0               |
| 1                                          | 3   | --   | --   | 50                                   | 67                   | 21                  | 53                              | 274                              | 0.5               |
| 1                                          | 3   | 0.25 | --   | 95                                   | 96                   | 21                  | 48                              | 269                              | 1.5               |
| 1                                          | 5   | --   | --   | 67                                   | 102                  | 15                  | 52                              | 327                              | 1.0               |
| 1                                          | 7.5 | --   | --   | 103                                  | 106                  | 20                  | 27                              | 278                              | 0.7               |
| 1.5                                        | 5   | 0.25 | --   | 140                                  | 149                  | 9                   | 357                             | 357                              | 2.8               |
| 2                                          | 1   | --   | --   | 29                                   | 50                   | 28                  | 52                              | 327                              | 4.4               |
| 2                                          | 1   | 0.25 | --   | 71                                   | 79                   | 27                  | 56                              | 154                              | 0                 |
| 2                                          | 2   | --   | --   | 41                                   | 60                   | 31                  | 24                              | 246                              | 0                 |
| 2                                          | 2   | 0.25 | --   | 90                                   | 90                   | 22                  | 52                              | 238                              | 2.1               |
| 2                                          | 3   | --   | --   | 61                                   | 74                   | 19                  | 50                              | 273                              | 1.0               |
| 2                                          | 3   | 0.25 | --   | 102                                  | 103                  | 19                  | 45                              | 246                              | 1.5               |
| 2                                          | 5   | --   | --   | 81                                   | 93                   | 18                  | 49                              | 315                              | 1.0               |
| 2                                          | 5   | 0.25 | --   | 140                                  | 151                  | 13                  | 46                              | 310                              | 1.3               |
| 2                                          | 5   | --   | 0.06 | 96                                   | 107                  | 13                  | 24                              | 323                              | 4.2               |
| 2                                          | 5   | --   | 0.16 | 126                                  | 133                  | 11                  | 42                              | 333                              | 2.2               |
| 2                                          | 5   | --   | 0.24 | 139                                  | 0                    | 1                   | 10                              | 392                              | 2.1               |
| 2                                          | 5   | --   | 0.25 | 134                                  | 1                    | 1                   | 10                              | 498                              | (1)               |
| 2.5                                        | 5   | --   | --   | 81                                   | 88                   | 14                  | 43                              | 421                              | (1)               |
| 2.5                                        | 5   | 0.25 | --   | 145                                  | 157                  | -----               | 15                              | 312                              | 1.6               |
| 2.5                                        | 7.5 | --   | --   | 94                                   | 101                  | 16                  | 42                              | 329                              | 4.2               |
| 2.5                                        | 10  | --   | --   | 107                                  | -----                | -----               | 408                             | 324                              | 1.8               |
| 3                                          | 1   | --   | --   | 38                                   | 57                   | 27                  | 48                              | 211                              | 1.5               |
| 3                                          | 1   | 0.25 | --   | 85                                   | 90                   | 19                  | 54                              | 278                              | 1.0               |
| 3                                          | 2   | --   | --   | 48                                   | 63                   | 21                  | 49                              | 235                              | 2.1               |
| 3                                          | 2   | 0.25 | --   | 96                                   | 96                   | 27                  | 55                              | 301                              | 1.0               |
| 3                                          | 3   | --   | --   | 70                                   | 82                   | 17                  | 44                              | 258                              | 1.5               |
| 3                                          | 3   | 0.25 | --   | 108                                  | 109                  | 17                  | 58                              | 329                              | 1.1               |
| 3                                          | 5   | 0.25 | --   | 139                                  | 149                  | 13                  | 27                              | 343                              | 4.2               |
| 3.5                                        | 5   | 0.25 | --   | 144                                  | 161                  | 11                  | 28                              | 355                              | 4.2               |
| 5                                          | 2   | --   | --   | 60                                   | 75                   | 20                  | 41                              | 250                              | 1.0               |
| 5                                          | 5   | --   | --   | 90                                   | 94                   | 12                  | 20                              | 312                              | 1.1               |
| 5                                          | 5   | 0.25 | --   | 144                                  | 147                  | 17                  | 24                              | 391                              | 2.3               |
| 5                                          | 7.5 | --   | --   | 109                                  | 118                  | 14                  | 26                              | 357                              | 0.7               |
| 7.5                                        | 7.5 | --   | --   | 116                                  | 116                  | -----               | 5                               | 391                              | (1)               |
| 7.5                                        | 5   | 0.25 | --   | 110                                  | 0                    | 1                   | 0                               | 398                              | 6.2               |
| 10                                         | 2   | --   | --   | 85                                   | 101                  | 13                  | 38                              | 302                              | 2.0               |
| 10                                         | 2   | 0.2  | --   | 123                                  | 127                  | 20                  | 39                              | 380                              | 1.5               |
| 10                                         | 2   | 0.20 | --   | 115                                  | 123                  | 15                  | 34                              | 376                              | 2.2               |
| 10                                         | 2   | --   | 0.2  | 135                                  | 142                  | 16                  | 30                              | 408                              | 2.1               |
| 15                                         | 2   | --   | --   | 107                                  | 109                  | 7                   | 26                              | 328                              | 1.7               |

<sup>1</sup> Brittle.

Table IV-A

[Commercial-Purity Ti-Sn-Al alloys]

| Composition, Percent<br>(Balance Titanium) |     | Tensile Properties: p. s. i. × 1,000 |                      |                     |                                 |                                  |                   |
|--------------------------------------------|-----|--------------------------------------|----------------------|---------------------|---------------------------------|----------------------------------|-------------------|
| Sn                                         | Al  | 0.2%<br>Offset<br>Yield              | Ultimate<br>Strength | Elongation<br>to 1" | Percent<br>Reduction<br>in Area | Annealed<br>Hardness,<br>Vickers | Min.<br>Bend<br>T |
| 1                                          | 5   | 49                                   | 76                   | 24                  | 44                              | 197                              | 1.3               |
| 1                                          | 5   | 106                                  | 116                  | 16                  | 38                              | 374                              | 2.7               |
| 2                                          | 5   | 114                                  | 122                  | 18                  | 39                              | 380                              | 2.5               |
| 2.5                                        | 5   | 106                                  | 114                  | 16                  | 41                              | 353                              | 1.7               |
| 3                                          | 5   | 108                                  | 114                  | 18                  | 40                              | 357                              | 3.3               |
| 4                                          | 5   | 115                                  | 118                  | 16                  | 31                              | 370                              | 5.7               |
| 5                                          | 1   | 74                                   | 87                   | 27                  | 44                              | 268                              | 1.8               |
| 5                                          | 1   | 83                                   | 92                   | 21                  | 58                              | 299                              | 1.7               |
| 5                                          | 3   | 92                                   | 102                  | 15                  | 28                              | 319                              | 2.8               |
| 5                                          | 3.5 | 103                                  | 121                  | 16                  | 24                              | 356                              | 3.6               |
| 5                                          | 4   | 104                                  | 122                  | 19                  | 34                              | 360                              | 2.7               |
| 5                                          | 4.5 | 117                                  | 124                  | 19                  | 49                              | 373                              | 2.2               |
| 5                                          | 5   | 120                                  | 125                  | 20                  | 47                              | 406                              | 2.5               |
| 9                                          | 1   | 86                                   | 99                   | 19                  | 42                              | 299                              | 1.7               |
| 9                                          | 2   | 99                                   | 109                  | 21                  | 46                              | 333                              | 2.7               |
| 9                                          | 3   | 110                                  | 118                  | 18                  | 33                              | 357                              | 2.5               |
| 9                                          | 3.5 | 120                                  | 132                  | 19                  | 33                              | 390                              | 2.5               |
| 9                                          | 4   | 125                                  | 132                  | 21                  | 40                              | 388                              | 4.6               |
| 9                                          | 4.5 | 131                                  | 131                  | 21                  | 46                              | 421                              | 2.3               |
| 9                                          | 5.0 | 127                                  | 137                  | 13                  | 30                              | 388                              | 3.0               |
| 13                                         | 1   | 112                                  | 122                  | 18                  | 26                              | 345                              | 2.5               |
| 13                                         | 2   | 124                                  | 124                  | 18                  | 30                              | 363                              | 2.6               |
| 13                                         | 3   | 135                                  | 135                  | 12                  | 25                              | 366                              | 5.1               |
| 13                                         | 2.5 | 134                                  | 138                  | 20                  | 36                              | 394                              | 2.5               |
| 13                                         | 4   | 143                                  | 146                  | 12                  | 27                              | 376                              | 4.8               |
| 13                                         | 4.5 | 146                                  | 149                  | 4                   | 18                              | 389                              | (1)               |
| 13                                         | 5   | 163                                  | 1                    | 1                   | 10                              | 422                              | (1)               |
| 16                                         | 1   | 97                                   | 131                  | 16                  | 21                              | 314                              | 1.8               |
| 16                                         | 2   | 133                                  | 145                  | 19                  | 30                              | 344                              | 2.4               |
| 16                                         | 3   | 152                                  | 164                  | 10                  | 19                              | 384                              | (1)               |
| 16                                         | 4   | -----                                | 148                  | 1                   | 5                               | 387                              | (1)               |
| 19                                         | 1   | 126                                  | 147                  | 14                  | 29                              | 329                              | 1.2               |
| 19                                         | 2   | 135                                  | 151                  | 7                   | 8                               | 342                              | 2.3               |
| 19                                         | 3   | 140                                  | 154                  | 4                   | 9                               | 372                              | (1)               |

<sup>1</sup> Brittle.

Table IV-B

[Commercial-purity Ti-Sn-Al alloys with interstitials]

| Composition, percent<br>(Balance Titanium) |    |      |      |    |                         | Tensile Properties: p. s. i. $\times 1,000$ |                          |                                 |                                  |        |
|--------------------------------------------|----|------|------|----|-------------------------|---------------------------------------------|--------------------------|---------------------------------|----------------------------------|--------|
| Sn                                         | Al | C    | O    | N  | 0.2%<br>Offset<br>Yield | Ultimate<br>Strength                        | Elonga-<br>tion<br>to 1" | Percent<br>Reduction<br>in Area | Annealed<br>Hardness,<br>Vickers | Bend T |
| 1                                          | 5  | 0.1  | --   | -- | 128                     | 133                                         | 16                       | 38                              | 422                              | 5.4    |
| 1                                          | 5  | 0.2  | --   | -- | 138                     | 143                                         | 14                       | 31                              | 451                              | 6.2    |
| 1                                          | 5  | 0.25 | --   | -- | 139                     | 144                                         | 20                       | 40                              | 444                              | 2.5    |
| 1                                          | 5  | --   | 0.1  | -- | 120                     | 129                                         | 16                       | 39                              | 393                              | 3.4    |
| 1                                          | 5  | --   | 0.2  | -- | 129                     | 136                                         | 21                       | 36                              | 431                              | 5.1    |
| 1                                          | 5  | --   | 0.1  | -- | 129                     | 135                                         | 14                       | 35                              | 384                              | 3.5    |
| 2                                          | 5  | 0.2  | --   | -- | 136                     | 141                                         | 18                       | 35                              | 423                              | 4.7    |
| 2                                          | 5  | --   | 0.1  | -- | 128                     | 136                                         | 12                       | 28                              | 437                              | 2.6    |
| 2                                          | 5  | --   | 0.2  | -- | 127                     | 133                                         | 17                       | 34                              | 423                              | 5.1    |
| 2.5                                        | 5  | 0.1  | --   | -- | 127                     | 134                                         | 16                       | 31                              | 394                              | 3.7    |
| 2.5                                        | 5  | 0.2  | --   | -- | 143                     | 147                                         | 19                       | 33                              | 438                              | 6.6    |
| 2.5                                        | 5  | --   | 0.2  | -- | 141                     | 143                                         | 22                       | 37                              | 422                              | 6.4    |
| 2.5                                        | 5  | --   | 0.1  | -- | 137                     | 142                                         | 16                       | 39                              | 423                              | 5.2    |
| 2.5                                        | 5  | --   | 0.2  | -- | 124                     | 131                                         | 3                        | 5                               | 421                              | 5.5    |
| 3                                          | 5  | 0.1  | --   | -- | 151                     | 155                                         | 5                        | 15                              | 442                              | (1)    |
| 3                                          | 5  | 0.2  | --   | -- | 138                     | 141                                         | 19                       | 33                              | 421                              | 4.8    |
| 3                                          | 5  | 0.25 | --   | -- | 140                     | 144                                         | 17                       | 29                              | 421                              | 4.5    |
| 3                                          | 5  | --   | 0.1  | -- | 142                     | 144                                         | 20                       | 35                              | 420                              | 2.7    |
| 3                                          | 5  | --   | 0.2  | -- | 132                     | 138                                         | 16                       | 40                              | 421                              | 5.2    |
| 3                                          | 5  | --   | 0.1  | -- | 139                     | 143                                         | 16                       | 31                              | 424                              | 5.1    |
| 3                                          | 5  | --   | 0.2  | -- | 122                     | 128                                         | 6                        | 12                              | 392                              | 5.6    |
| 3                                          | 5  | --   | 0.2  | -- | 148                     | 152                                         | 6                        | 15                              | 429                              | (1)    |
| 4                                          | 5  | 0.1  | --   | -- | 130                     | 134                                         | 20                       | 43                              | 405                              | 4.9    |
| 4                                          | 5  | --   | 0.2  | -- | 136                     | 137                                         | 2                        | 15                              | 428                              | 7.0    |
| 4                                          | 5  | --   | 0.1  | -- | 129                     | 134                                         | 12                       | 23                              | 404                              | 5.4    |
| 4                                          | 5  | --   | 0.2  | -- | 155                     | 156                                         | 2                        | 12                              | 454                              | (1)    |
| 5                                          | 1  | 0.2  | --   | -- | 105                     | 108                                         | 25                       | 50                              | 322                              | 1.2    |
| 5                                          | 1  | 0.2  | --   | -- | 105                     | 106                                         | 19                       | 42                              | 348                              | 3.3    |
| 5                                          | 1  | --   | 0.2  | -- | 127                     | 135                                         | 21                       | 38                              | 373                              | 2.0    |
| 5                                          | 2  | 0.2  | --   | -- | 118                     | 125                                         | 22                       | 49                              | 348                              | 2.4    |
| 5                                          | 2  | --   | 0.2  | -- | 117                     | 125                                         | 24                       | 40                              | 333                              | 2.4    |
| 5                                          | 2  | --   | 0.3  | -- | 125                     | 132                                         | 19                       | 40                              | 376                              | 2.4    |
| 5                                          | 3  | 0.2  | --   | -- | 125                     | 129                                         | 20                       | 46                              | 363                              | 1.9    |
| 5                                          | 3  | --   | 0.1  | -- | 125                     | 139                                         | 16                       | 31                              | 391                              | 4.8    |
| 5                                          | 3  | --   | 0.2  | -- | 124                     | 132                                         | 20                       | 41                              | 390                              | 2.2    |
| 5                                          | 3  | --   | 0.3  | -- | 131                     | 147                                         | 16                       | 31                              | 413                              | 6.6    |
| 5                                          | 3  | --   | 0.4  | -- | 151                     | 155                                         | 6                        | 12                              | 431                              | (1)    |
| 5                                          | 3  | --   | 0.20 | -- | 142                     | 146                                         | 15                       | 16                              | 417                              | 2.4    |
| 9                                          | 1  | 0.2  | --   | -- | 118                     | 123                                         | 23                       | 48                              | 357                              | 2.4    |
| 9                                          | 1  | --   | 0.2  | -- | 107                     | 118                                         | 9                        | 11                              | 380                              | 2.3    |
| 9                                          | 1  | --   | 0.15 | -- | 120                     | 128                                         | 9                        | 15                              | 373                              | 2.4    |
| 9                                          | 2  | 0.2  | --   | -- | 132                     | 136                                         | 16                       | 38                              | 380                              | 2.5    |
| 9                                          | 2  | --   | 0.2  | -- | 110                     | 117                                         | 5                        | 15                              | 376                              | 2.3    |
| 9                                          | 2  | --   | 0.16 | -- | 143                     | 148                                         | 20                       | 39                              | 390                              | 3.2    |
| 9                                          | 3  | 0.1  | --   | -- | 131                     | 142                                         | 16                       | 39                              | 401                              | 2.4    |
| 9                                          | 3  | 0.2  | --   | -- | 139                     | 142                                         | 16                       | 40                              | 397                              | 3.3    |
| 9                                          | 3  | 0.3  | --   | -- | 147                     | 156                                         | 23                       | 40                              | 418                              | 4.9    |
| 9                                          | 3  | 0.4  | --   | -- | 161                     | 163                                         | 19                       | 32                              | 450                              | (1)    |
| 9                                          | 3  | --   | 0.2  | -- | 130                     | 134                                         | 17                       | 28                              | 401                              | 3.3    |
| 9                                          | 3  | --   | 0.20 | -- | 148                     | 152                                         | 9                        | 14                              | (1)                              |        |
| 13                                         | 1  | 0.2  | --   | -- | 122                     | 148                                         | 13                       | 23                              | 390                              | 2.6    |
| 13                                         | 1  | 0.26 | --   | -- | 139                     | 144                                         | 22                       | 43                              | 383                              | 3.1    |
| 13                                         | 1  | --   | 0.2  | -- | 134                     | 140                                         | 15                       | 31                              | 376                              | 3.3    |
| 13                                         | 1  | --   | 0.14 | -- | 149                     | 151                                         | 16                       | 35                              | 413                              | 3.3    |
| 13                                         | 2  | 0.2  | --   | -- | 143                     | 153                                         | 18                       | 20                              | 411                              | 4.7    |
| 13                                         | 2  | --   | 0.2  | -- | 140                     | 150                                         | 4                        | 5                               | 386                              | 3.5    |
| 13                                         | 2  | --   | 0.16 | -- | 134                     | 154                                         | 9                        | 23                              | 387                              | 3.6    |
| 13                                         | 3  | 0.2  | --   | -- | 164                     | 164                                         | 12                       | 13                              | 416                              | (1)    |
| 13                                         | 3  | --   | 0.2  | -- | 156                     | 159                                         | 5                        | 13                              | 420                              | (1)    |
| 13                                         | 3  | --   | 0.22 | -- | 166                     | 166                                         | 0                        | 4                               | 331                              | (1)    |

<sup>1</sup> Brittle.

It is thus apparent that the ternary alloys of titanium with aluminum and tin, with or without the addition of interstitials, constitute an outstandingly versatile and desirable group, offering a wide range of properties and a composition tolerance for any given set of properties which greatly facilitates their production. Particularly desirable are the alloys containing 9% to 13% tin, 2% to 4% aluminum and about 0.2% carbon or another interstitial or combination of interstitials having a hardening and strengthening effect equivalent to that of 0.2% carbon.

The alloys of this invention, in general, will withstand prolonged aging at temperatures as high as 400° C. without material embrittlement—hence, they are particularly adapted for use under high temperature conditions. Moreover, these titanium-aluminum-tin alloys are susceptible to a variety of useful modifications by the addition of fractions of other metals. For example, some compositions are benefitted by the addition of 0.5% to 5% antimony. Typical alloys and their properties are:

| Composition, Percent<br>(Balance Titanium) |     |     |      | Tensile Properties: p. s. i. $\times 1,000$ |                       |                        |                      |                     |        |  |
|--------------------------------------------|-----|-----|------|---------------------------------------------|-----------------------|------------------------|----------------------|---------------------|--------|--|
| Al                                         | Sn  | Sb  | C    | V. H. N.<br>Surface                         | Proportional<br>limit | 0.2% Off-<br>set Yield | Ultimate<br>Strength | Elongation<br>in 1" | Bend T |  |
| 5                                          | 2.5 | 0.5 | 0.25 | 390                                         | 100                   | 150                    | 157                  | 14                  | 4.1    |  |
| 5                                          | 2.5 | 1.0 | 0.25 | 403                                         | 130                   | 137                    | 138                  | 17                  | 2.1    |  |
| 5                                          | 2.5 | 1.5 | 0.25 | 418                                         | 131                   | 143                    | 144                  | 5                   | (1)    |  |
| 5                                          | 2.5 | 2.5 | 0.25 | 392                                         | 129                   | 142                    | 143                  | 3                   | (1)    |  |
| 5                                          | 2.5 | 5   | 0.25 | 409                                         | 114                   | -----                  | 134                  | 1                   | (1)    |  |

<sup>1</sup> Brittle.

Beryllium in amounts from 0.1% to 1% is a useful addition, particularly for forging and cast-

titanium-aluminum-tin alloys containing 0.5% to 5% copper. The following are typical:

| Composition, Percent<br>(Balance Titanium) |     |     |      | Tensile Properties: p. s. i. $\times 1,000$ |                       |                        |                      |                     |        |  |
|--------------------------------------------|-----|-----|------|---------------------------------------------|-----------------------|------------------------|----------------------|---------------------|--------|--|
| Al                                         | Sn  | Cu  | C    | V. H. N.<br>Surface                         | Proportional<br>limit | 0.2% Off-<br>set Yield | Ultimate<br>Strength | Elongation<br>in 1" | Bend T |  |
| 5                                          | 2.5 | 0.5 | 0.25 | 404                                         | 100                   | 144                    | 156                  | 12                  | 4.1    |  |
| 5                                          | 2.5 | 1.0 | 0.25 | 407                                         | 124                   | 133                    | 133                  | 11                  | 2.5    |  |
| 5                                          | 2.5 | 1.5 | 0.25 | 424                                         | 130                   | 134                    | 134                  | 10                  | 3.6    |  |

ing alloys. Representative compositions and their properties are the following:

Manganese is a particularly desirable addition to a titanium-aluminum-tin base, being usable in

| Composition, Percent<br>(Balance Titanium) |     |      |      | Tensile Properties: p. s. i. $\times 1,000$ |                       |                        |                      |                     |        |
|--------------------------------------------|-----|------|------|---------------------------------------------|-----------------------|------------------------|----------------------|---------------------|--------|
| Al                                         | Sn  | Be   | C    | V. H. N.<br>Surface                         | Proportional<br>limit | 0.2% Off-<br>set Yield | Ultimate<br>Strength | Elongation<br>in 1" | Bend T |
| 5                                          | 2.5 | 0.1  | 0.25 | 396                                         | 133                   | 133                    | 138                  | 22                  | 4.0    |
| 5                                          | 2.5 | 0.25 | 0.25 | 409                                         | 136                   | 137                    | 139                  | 10                  | 3.8    |

Bismuth is useful when added in amounts from 0.5% to 5%, as shown by the following:

amounts from 0.25% to as high as 12%. Examples are as follows:

| Intended Composition,<br>Percent (Balance<br>Titanium) |     |     |      | Tensile Properties: p. s. i. $\times 1,000$ |                       |                        |                      |                     |        |
|--------------------------------------------------------|-----|-----|------|---------------------------------------------|-----------------------|------------------------|----------------------|---------------------|--------|
| Al                                                     | Sn  | Bi  | C    | V. H. N.<br>Surface                         | Proportional<br>Limit | 0.2% Off-<br>set Yield | Ultimate<br>Strength | Elongation<br>in 1" | Bend T |
| 5                                                      | 2.5 | 0.5 | 0.25 | 403                                         | 122                   | 131                    | 138                  | 15                  | 4.1    |
| 5                                                      | 2.5 | 1.0 | 0.25 | 387                                         | 128                   | 132                    | 133                  | 23                  | 2.3    |
| 5                                                      | 2.5 | 1.5 | 0.25 | 415                                         | 127                   | 141                    | 143                  | 3                   | (1)    |

<sup>1</sup> Brittle.

| Composition, Percent<br>(Balance Titanium) |    |     |      | Tensile Properties: p. s. i. $\times 1,000$ |                      |                     |                                   |        |  |
|--------------------------------------------|----|-----|------|---------------------------------------------|----------------------|---------------------|-----------------------------------|--------|--|
| Sn                                         | Al | Mn  | C    | 0.2% Off-<br>set Yield                      | Ultimate<br>Strength | Elongation<br>in 1" | Percent Red-<br>uction in<br>Area | Bend T |  |
| 2.5                                        | 5  | 0.5 | 0.25 | 133                                         | 133                  | 11                  | 21                                | 3.4    |  |
| 2.5                                        | 5  | 1   | 0.25 | 136                                         | 138                  | 13                  | 16                                | 4.0    |  |
| 2.5                                        | 5  | 1.5 | 0.25 | 151                                         | 152                  | 2                   | 2                                 | (1)    |  |
| 5                                          | 2  | 5   | --   | 140                                         | 145                  | 5                   | 26                                | 4.5    |  |
| 5                                          | 1  | 3   | --   | 138                                         | 145                  | 11                  | 35                                | 2.0    |  |
| 10                                         | 2  | 3   | --   | 164                                         | 164                  | 14                  | 47                                | 2.2    |  |
| 10                                         | 3  | 3   | --   | 179                                         | 181                  | 10                  | 34                                | 2.5    |  |
| 10                                         | 1  | 5   | --   | 149                                         | 156                  | 10                  | 41                                | 1.5    |  |
| 10                                         | 2  | 5   | --   | 162                                         | 167                  | 7                   | 13                                | 1.8    |  |
| 10                                         | 3  | 5   | --   | 181                                         | 185                  | 2                   | 8                                 | 6.2    |  |
| 10                                         | 1  | 7   | --   | 154                                         | 164                  | 8                   | 33                                | 2.5    |  |
| 10                                         | 2  | 7   | --   | 184                                         | 186                  | 5                   | 12                                | 6.5    |  |

<sup>1</sup> Brittle.

The properties of selected alloys of titanium, somewhat similar properties are found in aluminum, tin and silver are as follows, the silver being added up to about 10%:

| Composition, Percent<br>(Balance Titanium) |     |     |      | Tensile Properties: p. s. i. $\times 1,000$ |                       |                        |                      |                     |        |
|--------------------------------------------|-----|-----|------|---------------------------------------------|-----------------------|------------------------|----------------------|---------------------|--------|
| Al                                         | Sn  | Ag  | C    | V. H. N.<br>Surface                         | Proportional<br>limit | 0.2% Off-<br>set Yield | Ultimate<br>Strength | Elongation<br>in 1" | Bend T |
| 5                                          | 2.5 | 0.5 | 0.25 | 382                                         | 105                   | 130                    | 132                  | 22                  | 1.6    |
| 5                                          | 2.5 | 1.0 | 0.25 | 383                                         | 131                   | 132                    | 133                  | 20                  | 2.3    |

Zirconium is useful in amounts from 0.5% to about 20%, as exemplified by the following:

| Composition, Percent<br>(Balance Titanium) |     |     |      | Tensile Properties: p. s. i. $\times 1,000$ |                       |                        |                      |                     |            |
|--------------------------------------------|-----|-----|------|---------------------------------------------|-----------------------|------------------------|----------------------|---------------------|------------|
| Al                                         | Sn  | Zr  | C    | V. H. N.<br>Surface                         | Proportional<br>limit | 0.2% Off-<br>set Yield | Ultimate<br>Strength | Elongation<br>in 1" | Bend T     |
| 5                                          | 2.5 | 0.5 | 0.25 | 377<br>391                                  | 126<br>133            | 129<br>137             | 132<br>138           | 19<br>21            | 2.3<br>4.5 |

The aforesaid additions of one or more of antimony, beryllium, bismuth, copper, manganese, silver and zirconium are preferably alloyed with a titanium-tin-aluminum base containing about 1 to 5% tin, and 0.25 to 7.5% aluminum, and optimally about 3.5 to 7.5% aluminum. The added elements aforesaid retain the alpha structure of the base alloy with the exception of beryllium, copper and manganese. Beryllium forms intermetallic compounds. Copper and manganese are beta promoting or forming elements, depending on the amount added, in addition to which the beta phase promoted by copper precipitates an intermetallic compound during cooling much more so than the beta phase promoted by manganese.

The above described alloys comprising additions to the Ti-Al-Sn base of antimony, beryllium, bismuth, copper, manganese, silver and zirconium, are described and claimed in our co-pending applications Serial No. 294,263, filed June 18, 1952, and Serial No. 400,744, filed December 28, 1953, both comprising continuations-in-part of this application.

This application is a continuation-in-part of applicants' previously filed applications, Serial No. 151,314, filed March 22, 1950; Serial No. 209,905, filed February 7, 1951; Serial No. 253,564, filed October 27, 1951; and Serial Nos. 213,681 to 213,687, inc., all filed March 2, 1951. All of the above applications have become abandoned.

What is claimed is:

1. A titanium base alloy containing about: 1-23% tin, 0.25-7.5% aluminum, characterized in being ductile and forgeable and in having a tensile strength at least 10% in excess of the unalloyed titanium base metal.

2. An alloy consisting of about: 1-23% tin, 0.25-7.5% aluminum, up to 1% carbon, up to 0.5% oxygen, up to 0.3% nitrogen, and the balance titanium.

3. A titanium base alloy containing about:

1-23% tin, 0.25-7.5% aluminum, the tin content being related to the aluminum content with-

in said ranges, substantially in conformity with the following tabulation:

| Tin, Percent | Aluminum, Percent |
|--------------|-------------------|
| 1            | 0.5-6             |
| 5            | 0.5-5             |
| 10           | 0.5-4.5           |
| 15           | 0.25-4            |
| 20           | 0.25-3            |
| 23           | 0.25-1            |

characterized in being ductile and forgeable and in having a tensile strength at least 10% in excess of the unalloyed titanium base metal.

4. An alloy consisting of about 1-23% tin, 0.25-7.5% aluminum, the aluminum content being related to the tin content within said ranges, substantially in conformity with the following tabulation:

| Tin, Percent | Aluminum, Percent |
|--------------|-------------------|
| 1            | 0.5-6             |
| 5            | 0.5-5             |
| 10           | 0.5-4.5           |
| 15           | 0.25-4            |
| 20           | 0.25-3            |
| 23           | 0.25-1            |

said alloy also containing up to 1% carbon, up to 0.5% oxygen, up to 0.3% nitrogen, and the balance titanium.

ROBERT I. JAFFEE.  
HORACE R. OGDEN.  
DANIEL J. MAYKUTH.

References Cited in the file of this patent  
"The Canadian Mining and Metallurgical Bulletin," January 1950, page 27.  
"Journal of Metals," March 1950, page 498.